

Patented May 22, 1928.

1,671,070

# UNITED STATES PATENT OFFICE.

JOHN D. FORRESTER, OF KANSAS CITY, MISSOURI, ASSIGNOR TO PETER J. McINERNEY,  
OF DALLAS, TEXAS.

## PROCESS OF MAKING ASPHALTIC MATERIAL.

No Drawing.

Application filed June 26, 1925. Serial No. 39,815.

This invention relates to improvements for making asphaltic road material, and refers more particularly to a combination of an asphaltic binder and crushed stone adaptable for use both in the binder and surfacing courses of roads or streets.

Among the objects of the invention are to provide a process in which the asphaltic binder is intimately bonded to the crushed stone, a material which may be shipped in open-topped cars, easily loaded into and removed from the cars as distinguished from the usual type of asphaltic mixes which congeal and set, making it very difficult without the use of steam to unload asphaltic mixtures transported over any considerable distance.

Describing first the common type of binder course using crushed stone with an asphaltic binder, the crushed stone, termed as crusher run stone, is preferably limestone, granite or crushed gravel sized according to specification. Normally, for the binder course, stone ranging from one and one-fourth (1 1/4") inch to one-fourth (1/4") inch properly graded is satisfactory. With this is a filler of fine material of the same composition sufficiently small in size to pass a one-quarter inch screen and constituting substantially ten percent of the mix. With this is combined from 4% to 5% of asphaltic binder,—the same being thoroughly intermixed with the rock.

Material for the top course or wearing surface, varying somewhat in character from the binder course in that the crushed stone is of smaller size ranging from three-fourths inch to one-fourth inch properly graded material. With a top course the filler or fine material passing a one-fourth inch screen constitutes 20% of the mix and the asphaltic binder from 5% to 7%.

The asphalt specifications will vary with climatic conditions. Through the South, in States such as Texas, Alabama and Mississippi, the asphalt penetration will range from 60 to 70, while in the North, through Minnesota and the Dakotas, the penetration is normally in the neighborhood of 95. Ductility in all cases should not be under 85 at 77° F. This brief explanation of the characteristics of the binder and top courses used in connection with asphaltic highways, streets and roads, describes briefly the char-

acteristic of the particular ingredients or constituents of the road mix.

The greatest trouble experienced in handling material of this character and in laying asphaltic road mixes of this kind, is the fact that it can not be transported for any considerable distance from the plant where it is prepared without utilizing considerable heat in the way of steam for removing the mix from the cars due to the congealing of the asphalt and setting to form a tough solid mass. The present invention contemplates the transporting or conveying of such mixes, as described above, for considerable distances in railway cars, truck, or otherwise, due to the use of a liquefier or a relatively light solvent oil used with a mix for a double purpose, first, to carry the asphalt more effectively into the porous stone assuring a more satisfactory bond between the binder and crushed stone and at the same time maintaining the asphaltic binder in a more liquid or slushy condition over a considerable period of time prior to its evaporation facilitating the handling of the material until it can be rolled in place upon a highway or road.

It is recognized that at the present time this practice of using a liquefier or diluent vehicle is used in the preparation with a cold stone mix wherein the crushed rock is combined to the asphalt without heating the stone. In fact, at the present time two methods are employed for mixing crushed stone and asphalt as above described. In one case, a very satisfactory mix is prepared which is difficult to handle; in the other case, an easily handled mix is prepared which is not altogether satisfactory due to the lack of a proper bond between the asphaltic binder and the crushed stone.

Referring now to the first well known method of preparing this asphaltic material, crusher run stone is heated to 500° F. or more to eliminate the moisture. This heating is carried out in any suitable type of drier. The asphalt binder is then mixed therewith to thoroughly incorporate the bituminous substance with the crushed rock. The particular advantage of a mix of this character is the satisfactory and intimate bond which is effected between the asphaltic binder and the stone due to the removal of the moisture from the stone which increases

- its porosity and permits the liquid asphalt to penetrate more effectively into the surfaces of the rock. The disadvantage of this mixture is the difficulty in handling when 5 it has cooled due to the setting and congealing of the asphaltic binder into a tough solid mass which is impossible to handle except with a pick and can only be successfully removed from cars by the use of steam. An- 10 other difficulty is encountered in properly rolling this material in place on the road, as it necessitates relatively complete disintegration before the chunks of the material can be satisfactorily rolled.
- 15 A second well known manner of preparing an asphaltic crushed stone combination is that prepared under the name of "amesite" in which the stone is not heated but prepared and graded cold. To this stone is 20 added a liquefier which consists of relatively light oils or distillates having a Baumé gravity of 40° to 52°. To this combination is added the asphalt heated to a liquid condition. The liquefier, to a certain extent dis- 25 solving the asphalt, renders it more fluid and carries it into the stone to a certain limited extent. The cold stone containing considerable moisture has a retardent effect to the penetration of the asphaltic mate- 30 rial. The advantage of a mix of this character is, however, that it is easily worked and can be maintained over considerable periods of time in a relatively liquid slushy condition, thus rendering it especially adapt- 35 able to road work situated considerable distances from the plant in which it is mixed. This material can be shipped in open-topped cars to any part of the country and there easily unloaded if a liquefier is chosen which 40 evaporates slowly. It has been found that by carefully choosing a suitable liquefier and timing its evaporation period with the distance that the material is to be trans- 45 ported, a satisfactory mix which has the proper consistency on the job is produced. The disadvantage of a mix of this character, however, is that the presence of moisture in the cold stone prevents a satisfactory bonding or adhesion of the asphaltic binder to 50 the stone.
- 55 My present method is an improvement upon the above explained methods in that I heat the crusher run stone in a drier to a temperature of over 200° F., or in no event to a temperature more than 10° less than the flash point of the liquefier. In choosing a liquefier, or prime coat, I purposely select an oil having a gravity relatively the same as the solvent explained above, ranging 60 from 40° to 52° Baumé, but one which has a relatively high flash point in order to prevent flashing of the oil when combining the liquefier with the crushed stone. The heated rock, constituting properly graded 65 crushed stone with a filler such as described

in the first instance, is dumped into a pug mill or other type of mixer in which the liquefier is introduced. Asphalt heated to temperatures of from 250° to 325° F. is then added and thoroughly mixed to the combi- 70 nation of the crushed stone and liquefier. It is advisable that neither the crushed stone nor the asphalt be heated to the flash point of the liquefier. After thoroughly mixing the combination of the asphalt, crushed 75 stone and liquefier, a filler material, comprising not less than one-half percent or more than one percent of the total weight of the mix, is added. This filler material is preferably calcium hydrate or oxide, lime- 80 stone dust pulverized to the extent that it will pass a two hundred mesh screen, or hydraulic cement.

The particular advantages of preparing the mix in this manner are first there is 85 removed substantially all of the moisture from the stone which assures a better bonding between the asphaltic binder and the stone as the heat in removing the moisture increases the porosity of the stone. The 90 liquefier dissolves to a considerable extent the asphalt, reducing its surface tension and accelerates the penetration of the asphalt into the surface of the stone and the adhesion of the asphaltic binder to the stone, 95 effecting an intimate bond therebetween. It is particularly advantageous to select a liquefier which has a flash point above the boiling point of water in order that the moisture may be more effectively removed from 100 the stone without danger of flashing the liquefier. Also, a liquefier having a relatively high flash point permits the heating of the asphalt to a more fluid condition in which case it is more readily absorbed into 105 the surface of the stone. As described, a liquefier should be chosen where the mix is to be transported a short distance which will readily evaporate, while in the case where the mix is to be conveyed for a relatively 110 long distance from the plant in which it is prepared, a slowly evaporating liquefier is better adapted to such a mix as it maintains the crushed rock and asphalt combination in a slushy condition over a longer period of 115 time and prevents its congealing,—making it difficult to remove the mix from the cars in which it is transported.

While it is recognized that to heat crushed stone and combine it with asphalt or to use 120 a liquefier in preparing a cold crushed stone asphalt mix, is well known in the art, it is thought to be new to prepare a mix in the manner described, that is, heating the crushed stone to a temperature below the 125 flash point of the liquefier, combining the liquefier therewith, and adding an asphaltic binder, thus assuring a proper bonding of the asphaltic binder and crushed rock by elimination of the moisture in the rock and 130

effecting an easily workable mass by the use of a liquefier of the proper character.

The amount of liquefier used and the character of the liquefier will vary according to the particular asphalt and the character of the crushed stone as well as other varying conditions.

A further advantage of my process lies in the fact that a more uniform product is produced and better plant control may be had by drying all the crushed rock preliminarily to eliminate the moisture. Some rocks are notoriously deliquescent and rapidly acquire moisture in the atmosphere. Unless such materials are first heat treated or dried, the bonding of the asphalt is very unsatisfactory and stripping and peeling of the binder results.

Crushed stone aggregate is heated to temperatures of from 200° F. to 300° F. to substantially eliminate the moisture. To this hot stone is added a volatile oil liquefier, preferably in a closed retort, the liquefier having a flash point about the heat of the stone. Such a liquefier as naphtha, kerosene, light gas oil, or a combination of these oils, is satisfactory for this purpose. After being thoroughly combined with the heated rock, the bituminous or asphaltic composition which comprises an asphalt of from 60 to 95 penetration having a ductility normally not less than 85 at 77, is added, having first been sufficiently heated to facilitate its handling. This composition comprises of from 2.5% to 7% of the final mix.

I claim as my invention:

1. A process of making an asphaltic road mixture, comprising the steps of preparing the crushed stone aggregate by heating to a temperature to eliminate the moisture therefrom, adding to the crushed stone while hot a light oil having a flash point above the temperature of the drying heat and finally adding and thoroughly incorporating there-  
45 with an asphaltic binder.

2. A process of making an asphaltic road mixture adapted to be laid cold, comprising the steps of heating graded crushed stone in a drier to substantially eliminate the moisture therefrom, adding to the crushed stone while hot a hydrocarbon solvent thereto having a flash point above the temperature used in drying the stone and subsequently incorporating an asphaltic binder to produce a mix of easily workable consistency. 55

3. A process of making asphaltic road mixture adapted to be handled and laid cold and remaining at a workable consistency from the time of its preparation to its application, comprising the steps of heating crusher run stone in a drier to temperatures above the boiling point of water to substantially eliminate the moisture therefrom and increase the absorbent qualities thereof, adding to the crushed stone while hot a hydrocarbon solvent having a flash point above the temperature used in drying the stone and subsequently incorporating an asphaltic binder to produce a mix of a predetermined consistency, said solvent adapted to improve 70 the penetration and bonding effect of the binder with the stone.

4. A process for making an asphaltic road mixture, comprising the steps of drying the crushed stone by applying heat to remove 75 the moisture therefrom, adding a light solvent to the stone while in the heated state and subsequently adding an asphaltic binder.

5. A process for making an asphaltic road material comprising the steps of heating graded crushed stone in a drier to substantially eliminate the moisture therefrom, then adding to the crushed stone while in a heated condition a hydrocarbon solvent having a flash point above the drying temperature and subsequently incorporating an asphaltic binder to produce a mix of easily workable consistency. 85

JOHN D. FORRESTER.